

1

3,301,631

**PROCESS OF MODIFYING CELLULOSIC TEXTILES  
WITH EPIHALOHYDRIN-TRIAZONE REACTION  
PRODUCTS**

William L. Mauldin, Spartanburg, S.C., assignor to Deering Milliken Research Corporation, Spartanburg, S.C., a corporation of Delaware

No Drawing. Filed Aug. 21, 1962, Ser. No. 218,456

16 Claims. (Cl. 8—116.2)

This invention relates to methods for treating cellulosic textile materials to improve certain characteristics thereof, to the textile materials thus obtained and to novel compounds and compositions.

According to this invention, a cellulosic textile material as defined hereinafter, impregnated with a novel water-soluble reaction product of an epihalohydrin and a dimethylol-hydroxyalkyltriazole as defined hereinafter, is heated under textile resin curing conditions in the presence of an acid acting catalyst, to chemically fix the reaction product to the cellulosic material while the textile material is in a dry, unswollen condition. Preferably, the textile material is then contacted with strong aqueous base to further chemically fix the compound to the cellulosic material while the textile material is in a wet, swollen condition, thereby producing a product having further improved dry and wet resiliency, i.e., wrinkle resistance or recovery in both the wet and dry state. In a further improvement the textile material is contacted with both strong aqueous base and a wet cross-linking agent.

It is now well known that cellulosic materials can be treated with a textile resin to impart certain minimum care characteristics to fabrics produced from these textile materials. As a result of this textile resin treatment, fabrics having fairly satisfactory dry resiliency, i.e., good dry crease resistance or recovery, are presently being commercially produced in large quantities. It is characteristic of such fabrics, however, that they must normally be "drip dried," i.e., hung dripping wet after being washed, if the fabric is to have a semblance of a pressed appearance when dried. The reason for this is that although substantial dry resiliency can be imparted to the fabric, a lesser degree of wet resiliency, i.e., wet crease resistance or recovery, is imparted to the fabric by the resin treatment. It is impractical to attempt to overcome this deficiency by applying more resin as severe embrittlement or weakening of the material results along with other undesirable features such as a harsh, raspy hand and poor comfort values if the material is to be used in a garment.

By the process of this invention, it is now possible to produce fabrics having good wet as well as dry resiliency while at the same time retaining a higher percentage of the strength of the starting textile material than would be achieved with a conventional resin treatment, e.g., employing a known triazole. By this process, fabrics can be produced having at least as good residual strength and substantially better wet resiliency than is obtained by a conventional textile resin treatment. Frequently, fabrics having both increased residual strength and increased wet resiliency and about the same or greater dry resiliency can be obtained. Other properties are enhanced also, e.g., tear strength often is markedly increased over fabrics treated by a typical resin treatment.

It is therefore an object of this invention to provide a novel process for the production of textile materials having good wet and dry resiliency. It is another object to provide a novel process for the production of textile materials having a higher order of residual strength for any given degree of wet resiliency than can be obtained by a comparable resin treatment alone. It is a further

2

object to provide a novel treatment of textile materials. It is still another object to provide novel textile materials having good dry and wet resiliency. Another object is to provide novel chemically modified textile materials. Still another object is to provide novel compounds and compositions. Other objects will be apparent to those skilled in the art to which this invention pertains.

Textile materials which can be treated according to the process of this invention are those containing cellulosic fibers in which the anhydroglucose units are chemically substantially unmodified. Thus, the term "cellulosic textile material" when used herein means any textile material comprising fibers within the above definition, e.g., cotton, linen, jute, flax, regenerated cellulose fibers, including viscose rayon, in the form of staple, yarn and fabrics. This invention is directed primarily and preferably to cellulosic textile fabrics, including nonwovens, knitted and preferably woven fabrics. However, the advantages of this invention can be achieved by treating the 15 cellulosic fibers, yarns, or threads employed to produce these fabrics. The thus treated material, when woven or knitted into fabric will produce a fabric having better wet and dry resiliency than identical fabric woven from identical starting but untreated yarn or thread. Moreover, 20 the properties of the staple yarn and thread are modified in a desirable fashion. Satisfactory results can be achieved employing cellulosic materials containing both cellulosic and noncellulosic fibers, e.g., fabrics formed from a mixture of glycol-terephthalate, polyacrylic, or 25 nylon filaments or fibers with cotton or rayon can be improved by this process, preferably those whose cellulosic content of the fabric is substantial, e.g., about 40% or more by weight. As stated above, the invention is primarily directed to fabrics consisting essentially of cellulosic materials, especially cotton. Bleached and usually 30 also commercially mercerized or printed fabric, e.g., print-cloth, broadcloth, and oxfordcloth, is usually employed as the starting fabric. Generally, it is preferred to employ 35 starting fabrics having a tensile strength of at least 35 pounds and a tear strength of at least 400 grams in both 40 filling and warp directions.

The triazoles employed to produce the novel triazole-epihalohydrin reaction products are dimethylol-hydroxyalkyltriazole, dimethylol-hydroxyalkyl-thiatriazole and 45 the water-soluble ethers thereof. These known classes of compounds are prepared by reacting urea or thiourea with formaldehyde and a hydroxyalkylamine in about 1:4:1 molar ratios, respectively. If the ethers are desired, this 50 reaction can be conducted in the presence of two or more molar equivalents of the selected lower-alkanol or the dimethylol-hydroxyalkyl-triazole reacted subsequently with the lower-alkanol, all as is well known in the art.

The epihalohydrins employed to produce the novel triazole-epihalohydrin reaction products are epichlorohydrin, 55 epibromohydrin,  $\beta$ -methyl epichlorohydrin and other substituted epihalohydrins wherein one or more of the hydrogens of epichlorohydrin or epibromohydrin are substituted by a lower-alkyl group, e.g., methyl or ethyl, or an aryl group, e.g., phenyl.

The triazole-epihalohydrins employed in the process of this invention may thus be defined as the water-soluble 60 reaction product of an epihalohydrin and a triazole having the formula



wherein  $m$  is an integer from 2 to 8, preferably 2 to 4,  $n$  is an integer from 0 to 4, preferably 0 to 2, and  $X$  is oxygen or sulfur, preferably oxygen. These compounds are believed to be the result of the etherification of the hydroxy group of the hydroxyalkyl radical of the trizone by reaction with the epoxy group of the selected epihalohydrin. While this has not been conclusively proven, the resulting compound reacts with the cellulosic material in a typical textile resin fashion, thus indicating that the methyol groups are essentially unchanged. Also, active halogen, which can be titrated with strong base, is present in the trizone-epihalohydrin reaction product and in the cellulosic material which has been cured at an elevated temperature while impregnated with this reaction product and an acid acting textile resin catalyst, thus indicating that it is the epoxy group, rather than the halogen of the epihalohydrin which reacts with the starting trizone. This reactive halogen is chemically fixed to the resulting fabric, before it is contacted with strong base, as evidenced by the fact that it cannot be removed by washing with plain water.

If the above conclusions are correct, the trizone-epihalohydrin reaction products employed in the novel process have the formula



wherein  $m$ ,  $n$  and  $X$  have the values given above and  $\text{R}_1$ ,  $\text{R}_2$ ,  $\text{R}_3$ ,  $\text{R}_4$  and  $\text{R}_5$  are the groups present on the starting epihalohydrin, e.g., hydrogen, lower-alkyl, aryl, and  $\text{Hal}$  is chlorine or bromine. Examples of such compounds are the reaction product of epichlorohydrin and about a molar equivalent of dimethylol-hydroxyethyltriazone, epichlorohydrin and dimethylol- $\gamma$ -hydroxypropyl-triazone, epichlorohydrin and dimethylol- $\beta$ -hydroxypropyl-triazone, epichlorohydrin and dimethylol- $\beta$ -hydroxy- $\alpha$ -methylethyltriazone, epichlorohydrin and dimethylol-hydroxyethyl-thiotriazole, epichlorohydrin and dimethylol- $\gamma$ -hydroxypropyl-thiotriazole, and the dimethyl and the diethyl ethers of each of the above compounds.

These trizone-epihalohydrin reaction products are prepared by the reaction of the selected trizone (I) with an epihalohydrin. The reaction can be conducted in an inert organic solvent, in water or a lower-alkanol. The reaction will occur slowly at room temperature so elevated temperatures are preferred, e.g., 50°–100° C. The thus obtained product can then be diluted with water to provide the desired solids concentration. This reaction is apparently unique to a trizone having an N-hydroxyalkyl group attached as compounds such as dimethylol-ethyltriazone and ethylene-bis-dimethyloltriazone do not produce a comparable reaction product.

The molar ratio of epihalohydrin to trizone compound used to produce the reaction product employed in the process of this invention, is not critical, but best results are obtained when the molar ratio is about 1:1. The ratio can be varied from as low as 0.1:1 to 2:1 or higher, preferably 0.5:1 to 1.5, and more preferably 0.9:1 to 1.25:1. If more than a molar equivalent of epihalohydrin is employed, the excess ordinarily can be removed unchanged when the desired reaction is complete.

The amount of selected trizone-epihalohydrin reaction product which should be employed in the process of this invention will depend, of course, upon the amount of dry or wet crease resistance or resiliency desired in the treated textile material. Generally, from about 2% to about 25%, preferably 3% to 12%, and more preferably about 5% to 10%, is employed, calculated on the weight of the

dry textile material. As with conventional trizone treatment, an aqueous solution of the reaction product is ordinarily employed to impregnate the cellulosic material employing the concentration, usually between about 3% and 40%, which will provide the desired pickup on the selected textile material.

The textile resin catalysts employed during the heating step under textile resin curing conditions are a well-known class of compounds and include the "acid acting" compounds, i.e., those acidic in character under the curing conditions. The most common are the metal salts, e.g., magnesium chloride, zinc nitrate, and zinc fluoroborate, and the amine salts, e.g., monoethanolamine hydrochloride and 2 - amino - 2 - methyl - propanol nitrate. The amounts of catalyst to be employed are the same as those employed when using the usual textile resins, e.g., up to about 20% by weight of the trizone-epihalohydrin compound employed, with the preferred range being from about 0.5% to about 10%.

20 Other additives commonly employed when using the usual textile resins can be employed in the process of this invention. For example, a surfactant can be added to insure uniform and satisfactory wetting out of the fabric. Softeners, e.g., the dispersible polyethylenes, can be added to improve tear strengths when the textile material being treated is fabric.

In carrying out the heating, i.e., curing, step of the process of this invention the cellulosic material, uniformly impregnated with the selected trizone-epihalohydrin reaction product, is heated under textile resin curing conditions in the presence of an acid acting catalyst. Under ordinary conditions, this step employs conditions identical to that of a conventional resin treatment. For example, the selected reagents can be applied to the textile material 35 by padding, spraying, or applicator roll and then passed through squeeze rolls, if necessary to achieve the desired pickup of the reagents. Curing temperatures between 100° to 200° C., preferably about 140° to 190° C., are employed to chemically fix the reaction product to the textile material. When employing fabric these steps of 40 drying and curing are conducted while the fabric is free from extraneous wrinkles, usually in a smooth, open width condition. Conventional curing equipment is suitable for this operation. For example, when employing a fabric, 45 the reagents can be applied with the usual equipment and then passed through squeeze rolls and dried, e.g., at room temperature or while the fabric passes through a hot air oven or over heated cans. In production it is preferred to conduct the heating operations on fabric in a tenter frame to maintain the desired dimensions.

The thus treated textile material can then be given a thorough wash to remove the catalyst and any unreacted reagents, although such a step is not necessary.

As stated above, some of the advantages of this invention become apparent immediately after the reaction of the reaction product described with the cellulosic textile material under textile resin curing conditions. For example, greater residual strength is maintained in the fabric or an increase of at least one of dry and wet resiliency is observed, compared with an identical treatment employing the comparable trizone compound not reacted with an epihalohydrin. There are, however, reasons for employing the subsequent step of reacting the thus treated textile material with strong aqueous base. One of these is that an even greater degree of wet resiliency can be obtained after the second step without materially affecting the residual strength. The permanency of the treatment tends to be improved by the second step. Resistance to chlorine damage is often markedly improved by the second step.

The step of contacting the textile material with strong aqueous base employs conditions generally employed in the textile trade, and the necessary techniques will be apparent to those skilled in the art. For example, impregnating the textile material with the selected reagents can be accomplished in a manner similar to those employed

in the previous step. The material can be moistened by dipping in an aqueous solution of the selected base, squeezed through rollers to achieve the desired pickup of the base and then maintained at the selected temperature for a time sufficient to insure complete reaction, e.g., 1-24 hours, preferably 2-8 hours at 20-100° C., preferably about 50-90° C. The textile material is then preferably given a thorough wash to remove all reaction products not chemically fixed to the material.

The strong aqueous bases employed in the second step 10 of the preferred process of this invention are those having a pH of at least 10 as a 1% aqueous solution. The bases most commonly employed are the alkali-metal hydroxides, although other compounds such as sodium silicate and trisodium phosphate can also be employed. These bases are usually employed as about 0.2% to about 16% aqueous solutions, preferably about 2% to about 10%. The exact concentration, while not critical, will affect the results obtained. The concentration which gives the optimum result will depend, in part, on the percent pickup of the base by the textile material, the temperature at which the reaction is conducted, and the amount of base consumed in the reaction. Generally, the amount of base applied to the textile material should be at least the amount that will be consumed by the base reactive halogen group present in the triazole-epihalohydrin reaction product. Generally, a 1% to 10% aqueous solution of base is preferred when the wet pickup is between about 30% to 130%, calculated on the weight of the dry textile material.

While the wet configurational memory of the cured cellulosic material is improved by contacting it with strong base in the manner described above, even greater increases in wet configurational memory, as well as increases in dry configurational memory, are achieved if the cured material is contacted with both a strong aqueous base as defined above and a wet cross-linking agent, e.g., in the manner described in the application of D. M. Gagarine, S. N. 24,265, now U.S. Pat. No. 3,175,875, filed April 25, 1960, and in U.S. 2,985,501. "Wet cross-linking agent" means a polyfunctional agent which will cross-link the cured cellulosic material while it is in a hydrated state, usually in the presence of less than 130%, preferably less than 100%, e.g., 15-90%, moisture calculated on the weight of the dry cellulosic material. Wet cross-linking agents within the above general classification can be divided into three general classes. A first class comprises the polyepoxy cross-linking agents including diepoxybutane; the diglycidyl ether of ethylene glycol, propylene glycol, or diethylene glycol; the triglycidyl ether of glycerol; and the diglycidyl ether of bisphenol A; compounds having an  $\alpha$ -halohydrin group, e.g., chlorohydrin or bromohydrin, in place of one or more of the epoxy groups and compounds having a halogen atom, e.g., chlorine or bromine, on a carbon atom adjacent either an epoxy group or a halohydrin group. Examples of such latter compounds are epichlorohydrin, 1,3-dichloropropanol-2, 1,3-dibromopropanol-2, and bis-(1-chloro-2-hydroxy-n-propoxy)ethane. A second class of preferred alkaline catalyzed wet cross-linking agents include the sulfone activated divinyl compounds. Examples of this class of compounds are divinyl sulfone, bis-(vinyl sulfonyl) methane; and 1,4-bis-(vinyl sulfonyl)butane. A third class of alkaline catalyzed wet cross-linking agents are the carbonyl activated divinyl compounds, e.g., divinyl ketone, and octa-1,7-diene-3,6-dione. A fourth class are the carbonyl and sulfonyl activated sulfuric acid and phosphoric acid esters and their alkali-metal salts, e.g., disodium bisulfatoethyl sulfone.

The physical properties of the fabrics treated according to the process of this invention were determined according to accepted standard methods. Tear strength was determined by A.S.T.M. test designation D-1424-59. Tensile strength was determined by A.S.T.M. test designation D-39-59 (No. 10). Crease recovery angle was deter-

mined by A.S.T.M. test designation D-1295-53T. See "A.S.T.M. Standards for Committee D-13 on Textiles" (1959). Flat dry ratings were by A.A.T.C.C. test designation T-88-1958.

5 The following is illustrative of the processes and products of this invention, but is not to be construed as limiting.

#### Example I

In a 5 liter round bottom flask fitted with stirrer and condenser place 600 g. (10 moles) urea, 1200 g. (40 moles) of paraformaldehyde and 700 g. of dry methanol. To the stirred mixture slowly add 610 g. (10 moles) of ethanolamine. Stir until the mixture becomes homogeneous and then heat the mixture to 55° C. and add 920 g. (10 moles) of epichlorohydrin at a brisk rate to the thus produced dimethyl ether of dimethylol-hydroxyethyl-triazole. Heat the mixture at 80° C. for 3 hours. The thus produced product consists essentially of the dimethyl ether of N- $\beta$ -hydroxyethyl-dimethylol triazole-epichlorohydrin reaction product, pH 8.5, 68% cup solids, 22.6% water, Brookfield viscosity 130 c.p.s., 1.5 ml. 1 N H<sub>2</sub>SO<sub>4</sub> to neutrality.

#### Example II

25 Following the procedure of Example I, the N- $\beta$ -hydroxyethyl-dimethylol triazole-epichlorohydrin reaction product is prepared by substituting water for the methanol. This compound can also be prepared in a substantially anhydrous condition by removing the water azeotropically with benzene, followed by removal of the benzene prior to the addition of the epichlorohydrin. However, care must be exercised to prevent overheating during reaction with resulting product decomposition.

#### Example III

35 Following the procedure of Example I, the dimethyl ether of N- $\beta$ -hydroxyethyl-dimethylol thiotriazole-epichlorohydrin reaction product is prepared by substituting an equimolar amount of thiourea for the urea.

40 Any, or any combination of the following variations in the procedure of Example I can also be employed:

- (a) The methanol can be replaced by ethanol, propanol or butanol;
- (b) The amount of epichlorohydrin can be varied from 0.1 to 1.5 molar equivalents;
- (c) The epichlorohydrin can be replaced by epibromohydrin or  $\beta$ -methyl epichlorohydrin;
- (d) The ethanolamine can be replaced by an equimolar amount of 2-aminopropanol or 3-aminopropanol.

#### Example IV

50 Pass 39" 80 x 4.00 yd./lb. (in the greige) bleached and mercerized printcloth having 45 lbs. tensile and 450 g. tear (filling) into a pad bath containing either 10% 55 dimethylol-hydroxyethyl triazole (Rhonite N-17, Rohm & Haas, assuming 50% solids) or 15% of a triazole-epichlorohydrin reactant prepared in the manner of Example I using a 1:4:2.2:1:1 ratio of urea, paraformaldehyde, methyl alcohol, monoethanolamine and epichlorohydrin (equivalent to about 10% dimethylol-hydroxyethyl triazole) 1.5% Zn(NO<sub>3</sub>)<sub>2</sub>·6H<sub>2</sub>O, 2.5% formalin (to insure an excess of formaldehyde) and 0.35% Surfonic N-95 wetting agent. Adjust pickup to about 70%. Dry the fabric and cure in an oven at 350° F. for 1.5 minutes. Wash thoroughly.

65 Fabrics thus treated were found to have the properties shown in Table I.

TABLE I

| Reactant          | Spin | Tumble | Filling Tensile (lbs.) | Filling Tear (g.) |
|-------------------|------|--------|------------------------|-------------------|
| N-17.....         | 2.5  | 3.5    | 26                     | 260               |
| Triazole-epi..... | 3.8  | 5.0    | 27                     | 247               |

## Example V

Pad fabrics obtained according to the procedure of Example IV (without washing) with 5% aqueous KOH. Adjust wet pickup to about 70-75%. Roll up in a smooth roll, encase in a polyethylene bag and maintain at room temperature for 30 minutes. Wash the fabric thoroughly. Fabrics thus treated were found to have the properties shown in Table II.

TABLE II

| Reactant          | Spin | Tumble | Filling<br>Tensile<br>(lbs.) | Filling<br>Tear<br>(g.) |
|-------------------|------|--------|------------------------------|-------------------------|
| N-17-----         | 3.0  | 3.4    | 29                           | 220                     |
| Triazone-epi----- | 4.3  | 5.0    | 27                           | 240                     |

## Example VI

Pass 39" 80 x 80 4.00 yd./lb. (in the greige) bleached and mercerized printcloth having 49 lbs. tensile and 590 g. tear (filling) into a pad both containing either 5% or 10% solids (calculated on the basis of the starting hydroxyethyl triazone) of the triazone-epichlorohydrin reaction product of Example I, or 5% or 10% of dimethylol-hydroxyethyl-triazone (Rhonite N-17, Rohm & Haas, 50% solids assumed in the commercial product), in each case plus 1%, 1½% or 2%  $Zn(NO_3)_2 \cdot 6H_2O$  catalyst and 4% Moropol 700 emulsified polyethylene softener, and sufficient acetic acid to bring the pH of the bath to about 5. Adjust wet pickups to about 60-70%. (The percent of triazone-epichlorohydrin reactant was calculated on the basis of the starting triazone, rather than the product so that the comparison would be on a molar rather than weight basis.) Dry the impregnated fabric on dry cans heated with steam at 17 p.s.i. and then cure at 350° F. for 1.5 minutes. Impregnate portions of each of the thus treated fabrics with 2.5% aqueous NaOH with a wet pickup of about 70%, followed by about an 8 to 12% add-on of epichlorohydrin, calculated on the dry weight of the fabric, applied by means of an applicator roll. Roll up the wet fabric on rolls and wrap in polyethylene film and then age for two hours at 160° F. Give all fabric samples a standard wash with detergent in an automatic washer and dry.

Fabric thus treated was submitted for testing. The results of these tests are shown in Table III.

By comparing Sample 4 with 3 and 1, 8 with 7 and 5, 12 with 11 and 9, 16 with 15 and 13, 20 with 19 and 17, and 24 with 23 and 21, it can be seen that when fabric treated with the triazone-epichlorohydrin reactant followed by NaOH-epi is obtained which has about the same tensile and tear properties as fabric treated with the triazone, with or without the second NaOH-epi treatment, the triazone-epichlorohydrin treated fabric will have substantially better spin performance than the triazone treated fabric. Conversely, if about the same spin performance is achieved in the two types of fabrics, the triazone-epichlorohydrin treated fabric will have substantially higher tensile and tear strength.

## Example VII

Follow the procedure of Example VI, but substitute the dimethylol-hydroxyethyl-triazone epichlorohydrin reaction product produced according to the procedure of Example II for the corresponding dimethyl ether employed in Example VI. The thus obtained fabric has substantially the same properties as that obtained according to the procedure of Example IV.

## Example VIII

Follow the procedure of Example VI, but substitute the dimethyl ether of  $N$ - $\beta$ -hydroxyethyl-dimethylol-thiotriazone-epichlorohydrin reaction product obtained according to the procedure of Example III. Fabric thus obtained has substantially the same properties as that obtained according to the procedure of Example I.

It has been noted that fabrics treated with a reactant of this invention has a tendency to pick up soil when washed with very dirty materials. Surprisingly, this tendency can be virtually eliminated if the fabric is impregnated with a sulfonic acid, preferably an aromatic mono or poly sulfonic acid. For example, fabric obtained following the procedure of Example VI showed a pronounced tendency to pick up soil from dirty water. However, if the fabric is padded with, e.g., a 1-10% aqueous solution of Erion N. W., the mixed condensation product of naphthalene sulfonic acid, dihydroxy-diphenyl sulfones and formaldehyde, and then heated, preferably at a temperature of at least 140° F., this tendency is substantially eliminated. Other compounds which can be used are the sulfonic acid group containing synthetic tanning agents, e.g., the condensation product formaldehyde and naphthalene sulfonic acid, formaldehyde and phenol sulfonic acid, formalde-

TABLE III

| Reactant                 | Before or after<br>NaOH-epi<br>treatment | Sample<br>No. | 5% reactant pickup* |        |                              |                      | Sample<br>No. | 10% reactant pickup* |        |                              |                      |
|--------------------------|------------------------------------------|---------------|---------------------|--------|------------------------------|----------------------|---------------|----------------------|--------|------------------------------|----------------------|
|                          |                                          |               | Spin                | Tumble | Filling<br>tensile<br>(lbs.) | Filling<br>tear (g.) |               | Spin                 | Tumble | Filling<br>tensile<br>(lbs.) | Filling<br>tear (g.) |
| 350° Cure, 1% Catalyst   |                                          |               |                     |        |                              |                      |               |                      |        |                              |                      |
| Triazone-----            | Before                                   | 1             | 3.4                 | 3.9    | 28.3                         | 407                  | 5             | 3.5                  | 5.0    | 25.3                         | 340                  |
| Triazone-epi-----        | do                                       | 2             | 2.5                 | 3.4    | 31.5                         | 413                  | 6             | 3.0                  | 4.4    | 31.5                         | 447                  |
| Triazone-----            | After                                    | 3             | 3.9                 | 4.3    | 23.5                         | 367                  | 7             | 3.8                  | 4.8    | 24.0                         | 310                  |
| Triazone-epi-----        | do                                       | 4             | 4.5                 | 4.0    | 25.0                         | 373                  | 8             | 3.7                  | 4.5    | 30.2                         | 380                  |
| 350° Cure, 1.5% Catalyst |                                          |               |                     |        |                              |                      |               |                      |        |                              |                      |
| Triazone-----            | Before                                   | 9             | 2.8                 | 3.8    | 27.7                         | 400                  | 13            | 3.7                  | 4.9    | 26.5                         | 333                  |
| Triazone-epi-----        | do                                       | 10            | 3.2                 | 3.6    | 29.3                         | 413                  | 14            | 2.7                  | 4.4    | 32                           | 440                  |
| Triazone-----            | After                                    | 11            | 4.1                 | 4.0    | 23.3                         | 340                  | 15            | 4.9                  | 5.0    | 21.7                         | 300                  |
| Triazone-epi-----        | do                                       | 12            | 4.6                 | 4.1    | 21.8                         | 320                  | 16            | 4.3                  | 4.6    | 26.7                         | 347                  |
| 350° Cure, 2% Catalyst   |                                          |               |                     |        |                              |                      |               |                      |        |                              |                      |
| Triazone-----            | Before                                   | 17            | 2.3                 | 3.7    | 24.2                         | 360                  | 21            | 3.8                  | 4.7    | 26.0                         | 310                  |
| Triazone-epi-----        | do                                       | 18            | 3.4                 | 4.5    | 23.8                         | 367                  | 22            | 2.0                  | 4.3    | 26.5                         | 427                  |
| Triazone-----            | After                                    | 19            | 3.7                 | 4.1    | 22.0                         | 327                  | 23            | 4.0                  | 5.0    | 24.8                         | 330                  |
| Triazone-epi-----        | do                                       | 20            | 4.1                 | 4.5    | 25.3                         | 360                  | 24            | 4.5                  | 4.6    | 27.8                         | 360                  |

\*The percent of triazone-epichlorohydrin reactant was calculated on the basis of the starting triazone reactant.

hyde and naphthol sulfonic acid, the sulfonic acid group containing colorless dyes, i.e., whiteners or brighteners, e.g., Lucophor A, Blancophor ES-31, Calcophor white ST, Uvitex CF, Hiltamine arctic white CC, and other inorganic and organic sulfonic acids, e.g., sulfamic acid, the benzyl ether of 1-naphthol-3,6-disulfonic acid, both in the acid and alkali-metal forms. Preferably, the treatment is conducted at an acid pH.

What is claimed is:

1. A method for improving the properties of a cellulosic textile material containing at least 1.8 free hydroxy groups per anhydroglucose unit which comprises curing said material, impregnated with a water-soluble reaction product of an epihalohydrin and a triazone having the formula



wherein  $m$  is an integer from 2 to 8, inclusive,  $n$  is an integer from 0 to 4, inclusive, and  $X$  is selected from the group consisting of oxygen and sulfur, at an elevated temperature in the presence of an acid acting catalyst, and then contacting the material with a strong base under aqueous conditions until reaction with the base reactive halogens on said material is substantially complete.

2. A method according to claim 1 wherein the epihalohydrin is epichlorohydrin.

3. A method according to claim 1 wherein  $X$  is oxygen and  $m$  is 2.

4. A method according to claim 1 wherein the cellulosic material is cotton fabric.

5. A method according to claim 1 wherein a wet cross-linking agent is applied to the material along with the strong base.

6. A method according to claim 5 wherein the wet cross-linking agent is epichlorohydrin.

7. A method for improving the properties of a cellulosic textile fabric whose cellulosic content contains at least 1.8 free hydroxy groups per anhydroglucose unit which comprises the steps of applying to said fabric a water-soluble reaction product of between about 0.1 and about 1.5 moles of epichlorohydrin and a hydroxyethyl triazone having the formula



wherein  $n$  is an integer from 0 to 2, inclusive, curing said reaction product on said fabric at an elevated temperature in the presence of an acid acting catalyst, and thereafter applying an aqueous solution of at least a molar equivalent, calculated on the reaction product, of an alkali-metal hydroxide to the resulting fabric until reaction with the base reactive halogens on said fabric is substantially complete.

8. A method according to claim 7 wherein the fabric is cotton.

9. A method according to claim 7 wherein the reaction product is that of about one molar equivalent of epichlorohydrin and triazone are utilized, and wherein  $n$  is 1.

10. A method according to claim 7 wherein the reaction product is that of about one molar equivalent of epichlorohydrin and triazone are utilized, and wherein  $n$  is 0.

11. A method according to claim 8 wherein a wet cross-linking agent is applied to fabric along with the strong base.

12. A method according to claim 11 wherein wet cross-linking agent is epichlorohydrin.

13. A method for improving the properties of a cellulosic textile material containing at least 1.8 free hydroxy groups per anhydroglucose unit which comprises curing said material, impregnated with a water-soluble reaction product of an epihalohydrin and a triazone having the formula



wherein  $m$  is an integer from 2 to 8, inclusive,  $n$  is an integer from 0 to 4, inclusive, and  $X$  is selected from the group consisting of oxygen and sulfur, at an elevated temperature in the presence of an acid acting catalyst.

14. The product of the method of claim 13.

15. The product of the method of claim 1.

16. The product of the method of claim 7.

#### References Cited by the Examiner

#### UNITED STATES PATENTS

|              |         |          |       |         |
|--------------|---------|----------|-------|---------|
| 2,615,888    | 10/1952 | Zerner   | ----- | 260—248 |
| 2,892,674    | 6/1959  | Sause    | ----- | 8—116.2 |
| 2,950,553    | 8/1960  | Hurwitz  | ----- | 8—116.3 |
| 50 2,985,501 | 5/1961  | Gagarine | ----- | 8—120   |
| 3,014,907    | 12/1961 | Kober    | ----- | 260—248 |
| 3,016,281    | 1/1962  | Kropa    | ----- | 8—116.2 |
| 3,053,798    | 9/1962  | D'Alelio | ----- | 260—248 |

55 NORMAN G. TORCHIN, Primary Examiner.

JULIAN S. LEVITT, Examiner.

J. CANNON, Assistant Examiner.